

## UNITED STATES PATENT OFFICE

JAMES BADDILEY, OF BLACKLEY, MANCHESTER, ENGLAND, ASSIGNOR TO BRITISH DYESTUFFS CORPORATION LIMITED, OF BLACKLEY, MANCHESTER, ENGLAND

## PROCESS OF DYEING

No Drawing. Application filed May 26, 1927, Serial No. 194,542, and in Great Britain September 7, 1926.  
Renewed September 24, 1929.

By this invention, regenerated cellulose silks, such as viscose silk, are dyed in level shades with the monoazo dyestuffs obtained on coupling diazotized aromatic amines, their homologues, derivatives, and the sulphonlic acids and carboxylic acids thereof, for instance aryl amines having the general formula  $H_2N-R$ , wherein  $R_1$  represents a phenyl or naphthyl residue or the alkyl, nitro, chloro, sulphonlic or carboxylic derivatives of such residue, with a 2-amino-5-naphthol-7-sulphonlic acid, including in this expression its N-substituted derivatives. Some of the dyestuffs of this class are already known but they have never been used commercially, probably because they possess too small an affinity for cotton. I have now made the entirely unexpected discovery that these dyestuffs possess a good affinity for regenerated cellulose silks and in particular that they give level dyeings on these fibres. It is now well known that the regenerated cellulose silks generally possess a very uneven avidity for the usual cotton colours, which causes the dyeings obtained to be unlevel. My discovery of a range of dyestuffs which give even dyeings on these fibres is therefore of considerable value to those engaged in the process of dyeing regenerated cellulose silks.

The regenerated cellulose silk materials are dyed in the usual way. The following description is typical of the manner in which the dyeing may be carried out, but it must be understood that these conditions may be varied considerably and that I do not limit myself to the conditions given in the example.

*Example*

The dyebath is made up from 3,000 parts of water and 1 part of the dyestuff produced by combining the diazo compound of  $\beta$ -naphthylamine with 2-benzoylaminio-5-naphthol-7-sulphonlic acid. 100 parts of the regenerated cellulose silk material are entered into the dyebath, which is then brought to the boil. About 10 parts of Glauber's salt or common salt are then added and dyeing allowed to proceed at or near the boil for half to three-quarters hours. If desired, soap may be added

to the dyebath. The fabric is dyed a bright red shade, the dyeing being particularly level.

The following further examples illustrate the shades I obtain according to this invention, the dyeing being carried out in the usual way.

| Monoazo dyestuff from:-                                               |                                                  | Shade on viscose silk | 60  |
|-----------------------------------------------------------------------|--------------------------------------------------|-----------------------|-----|
| Amino compound diazotized                                             | Second component                                 |                       |     |
| $\beta$ -naphthylamine                                                | 2-amino-5-naphthol-7-sulphonlic acid             | Scarlet               |     |
| 2-naphthylamine-6-sulphonlic acid                                     | 2-amino-5-naphthol-7-sulphonlic acid             | Scarlet               |     |
| p-chloroaniline                                                       | 2-ethylamino-5-naphthol-7-sulphonlic acid        | Scarlet               | 65  |
| Aniline                                                               | 2-phenylamino-5-naphthol-7-sulphonlic acid       | Scarlet               |     |
| o-anisidine                                                           | 2-phenylamino-5-naphthol-7-sulphonlic acid       | Scarlet               |     |
| p-aminoacetanilide (the acetyl group being hydrolyzed after coupling) | 2-phenylamino-5-naphthol-7-sulphonlic acid       | Violet                | 70  |
| Dehydrothio-p-toluidine-sulphonlic acid                               | 2-phenylamino-5-naphthol-7-sulphonlic acid       | Crimson               |     |
| o-anisidine                                                           | 2-p-tolylamino-5-naphthol-7-sulphonlic acid      | Red                   | 75  |
| p-chloroaniline                                                       | 2-o-anisylamino-5-naphthol-7-sulphonlic acid     | Red                   |     |
| p-chloroaniline                                                       | 5-hydroxy-2,2'-dinaphthylamine-7-sulphonlic acid | Red                   | 80  |
| 2-chloro-4-amino-1-methylbenzene-5-sulphonlic acid                    | 5-hydroxy-2,2'-dinaphthylamine-7-sulphonlic acid | Bluish-red            |     |
| Aniline                                                               | 2-benzoylaminio-5-naphthol-7-sulphonlic acid     | Orange                | 85  |
| $\beta$ -naphthylamine                                                | 2-benzoylaminio-5-naphthol-7-sulphonlic acid     | Red                   |     |
| p-nitroaniline                                                        | 2-benzoylaminio-5-naphthol-7-sulphonlic acid     | Orange                | 90  |
| m-aminobenzoic acid                                                   | 2-benzoylaminio-5-naphthol-7-sulphonlic acid     | Orange                |     |
| 2-naphthylamine-6,8-disulphonlic acid                                 | 2-benzoylaminio-5-naphthol-7-sulphonlic acid     | Pink                  | 95  |
| p-chloroaniline                                                       | 2-benzoylaminio-5-naphthol-7-sulphonlic acid     | Orange                |     |
| Aniline                                                               | 5-hydroxy-2-naphthylglycine-7-sulphonlic acid    | Orange                | 100 |

5-hydroxy-2:2'-dinaphthylamine-7-sulphonic acid does not appear to have been previously described. It is prepared by heating 2-amino-5-naphthol-7-sulphonic acid with sodium bisulphite and  $\beta$ -naphthylamine.

- 5 When the reaction is completed, the mixture is diluted and the product precipitated by the addition of common salt, filtered off, dissolved in soda and filtered from unchanged  $\beta$ -naphthylamine and any  $\beta\beta$ -dinaphthylamine which may be present. The 5-hydroxy-2:2'-dinaphthylamine-7-sulphonic acid is then precipitated as white or greyish substance by acidifying the filtrate.

10 What I claim and desire to secure by Letters Patent is:—

1. The process of dyeing regenerated cellulose material in level shades characterized by the application to the material of monoazo dyestuffs obtained by coupling a 2-paratolylamino-5-naphthol-7-sulphonic acid with a diazo compound.

2. The process of dyeing regenerated cellulose material in level shades characterized by the application to the said material of monoazo dyestuffs obtained by coupling a sulphonated amino naphthol of the following structure



35 where R represents hydrogen, an alkyl or acyl group, or a phenyl or naphthyl residue, with a diazo compound.

- 40 3. Regenerated cellulose materials dyed in level shades by the application to the material of monoazo dyestuffs obtained by coupling a sulphonated amino naphthol of the following structure



50 where R represents hydrogen, an alkyl or acyl group, or a phenyl or naphthyl residue, with a diazo compound.

- 55 4. The process of dyeing regenerated cellulose material in level shades characterized by the application to the said material of monoazo dyestuffs obtained by coupling a sulphonated amino naphthol of the following structure



65 wherein R represents hydrogen, an alkyl or acyl group, or a phenyl or naphthyl residue, with a diazotized aryl amine having the formula  $H_2N-R_1$  wherein  $R_1$  represent a

phenyl or naphthyl residue or the alkyl, nitro, chloro, sulphonic or carboxylic substituted derivatives of such residue.

- 70 5. Regenerated cellulose materials dyed in level shades by the application to the material of monoazo dyestuffs obtained by coupling a sulphonated amino naphthol of the following structure



80 wherein R represents hydrogen, an alkyl or acyl group, or a phenyl or naphthyl residue, with a diazotized aryl amine having the formula  $H_2N-R_1$  wherein  $R_1$  represents a phenyl or naphthyl residue or the alkyl, nitro, chloro, sulphonic or carboxylic substituted derivatives of such residue.

85 In testimony whereof I affix my signature.

JAMES BADDILEY.

90

95

100

105

110

115

120

125

130